

Feb. 7, 1933.

A. H. HEYROTH

1,897,004

ELECTRICAL CONNECTION FOR NONMETALLIC RESISTORS

Filed Jan. 19, 1931

2 Sheets-Sheet 1

*Fig. 1.*



*Fig. 2.*



INVENTOR  
ALBERT H. HEYROTH

BY *R. B. Bemmer.*

ATTORNEY

Feb. 7, 1933.

A. H. HEYROTH

1,897,004

ELECTRICAL CONNECTION FOR NONMETALLIC RESISTORS

Filed Jan. 19, 1931

2 Sheets-Sheet 2



*Fig. 4.*



INVENTOR  
ALBERT H. HEYROTH

BY *R. B. Bemner*

ATTORNEY

## UNITED STATES PATENT OFFICE

ALBERT H. HEYROTH, OF NIAGARA FALLS, NEW YORK, ASSIGNOR TO THE GLOBAR CORPORATION, OF NIAGARA FALLS, NEW YORK

## ELECTRICAL CONNECTION FOR NONMETALLIC RESISTORS

Application filed January 19, 1931. Serial No. 508,598.

The invention relates to electric furnaces having rigid non-metallic resistors and to improved methods of making electrical connections therein. The invention is particularly applicable to furnaces employing silicon carbide resistors.

In the use of silicon carbide resistors the elements can be placed directly within the furnace chamber, and it is customary to make electrical contact by means of metallic terminal members extending through the furnace wall. These terminals also function as a means of support for the element, and are so positioned that the metallic surface in contact with the end of the resistor is comparatively close to the inner wall of the furnace chamber. In high temperature furnaces the metal is thus exposed to intense heat and, in addition, there is always considerable arcing at the points of areas of contact with the resistor.

If it were attempted to operate a metallic contact of this character without water cooling, the terminal would have a very short life. On the other hand, the introduction of water cooling causes considerable heat loss, since the terminal extends into the hotter portion of the furnace. Measurements made have shown that the heat loss due to water cooling may be an appreciable part of the total power consumed.

In the electric furnaces described herein, I employ two or more rigid non-metallic resistors, and make electrical connections between the ends of two adjacent resistors by means of a conducting material which is sufficiently refractory so that it can be placed entirely within the furnace chamber. Owing to the fact that silicon carbide resistors are operated in air without protection from oxidation, oxidizable materials such as carbon and graphite, which are both highly conducting and refractory, cannot be used. Metals are also impractical when placed entirely within the furnace because of their comparatively low melting points, their oxidizability and their inability to withstand the arcing which takes place at the ends of the resistor. I have found that a connector composed of a material which

I will designate as a siliconized silicon carbide can be placed entirely within the furnace chamber without causing deterioration of the contact. A furnace containing such a connecting member can be operated for prolonged periods of time at temperatures up to 1400 degrees centigrade without appreciable oxidation of the contact material. The electrical conductivity of the siliconized material is sufficiently great in comparison with that of the resistor so that very little heat is generated by the passage of the current through the terminal or connecting members. The size of the connectors can also be regulated so as to afford a minimum of electrical resistance.

The introduction of a connecting member which can be placed entirely within the furnace chamber makes possible the connection of two or more resistors in series with only half the usual number of external terminals. If water cooled metal terminals are used for the external contacting members, the heat loss caused by water cooling is reduced to half of that which would otherwise obtain. The element and the connecting members are much more readily replaced than is the case when the usual terminal mounting is employed at each end of the resistor.

In many furnace installations employing external terminals for each end of the resistor, the terminal mountings are either inaccessible or occupy space which could be advantageously used for other purposes. As examples of such installations, there are many furnaces where the silicon carbide rods are positioned vertically, and the terminals are placed underneath the furnace, and in other installations it is necessary to place the terminal mountings in the rear of the furnace or adjacent to one of the walls of the room. If an internal connector is used, the connecting member can be readily replaced, and the external connecting members are always accessible since they are placed on one side of the furnace only.

The nature of my improved contacting members and the method of employing them will be evident from the accompanying drawings, in which

55

60

65

70

75

80

85

90

95

100

Figure 1 shows a sectional view of an electric furnace in which two resistor elements are connected in series by means of a siliconized silicon carbide connector;

5 Figure 2 shows a section of the furnace shown in Figure 1, the section being taken along the lines II-II;

10 Figure 3 shows a sectional view of a furnace in which the elements are mounted vertically, the internal connector resting on the floor of the furnace and being readily replaceable; and

15 Figure 4 shows a sectional view of a muffle furnace in which the resistors are placed outside the heating chamber and the resistors connected by means of a connector at the rear of the furnace.

20 Referring to Figures 1 and 2, the silicon carbide resistors 1 are supported by resilient butt-end engagement with the terminal members 2. These terminal members may be water cooled as indicated, the inlet and outlet passages connected with the water system being designated by 3 and 4 respectively.

25 The inlet passage 3 is connected with the tube 9 so that the cooling fluid impinges upon the metal terminal facing 8. The water connections are made through the cap 5 which forms the extremity of the terminal. Pressure

30 against the ends of the silicon carbide resistors is afforded by the springs 12. The terminal members 2 furnish a means both for support and electrical connection. The siliconized silicon carbide connector 6 can be rigidly

35 attached to the furnace wall or, if desired, can be supported by the pressure exerted through the resistor; however, it is desirable that the connector fit into a cavity in the furnace wall and project somewhat from the sur-

40 face of the wall in order that the connector can be readily removed if necessary. It is desirable that the connectors be provided with recesses 7 for engagement with the ends of the resistors.

Any method of resilient mounting can be used for positioning the external terminals and for affording pressure against the ends of the resistor rods. In the method shown in Figure 2, the lever 10 is forced against the 50 terminal 2 by means of the spring 12. The lever 10 possesses a recessed portion 11 at the opposite end from the portion adapted to engage with the terminal member 9. This recessed portion 11 engages with the bracket 13, which is mounted on the wall of the furnace. The effect is thus the same as if the lever 10 were pivoted at the recessed portion 11. The metal terminal facing 8 is recessed at 15 so as to engage with the end of the resistor 1. The recess may be either cup shaped or conical. A refractory tube 16 may be used as a bushing for the terminal.

With the connector shown in Figure 3, the projecting portions 18 are adapted to fit into corresponding cavities in the bottom of the

furnace. The connector is thus positioned with respect to the floor of the furnace, and at the same time can be readily replaced.

70 In the use of silicon carbide resistors, it is occasionally desired to place the elements outside of the chamber containing the ware, in order to effect a more uniform distribution of heat, or to protect the resistor from injurious substances present within the heating chamber. In such cases, it is also advantageous to use a siliconized silicon carbide connector to eliminate a portion of the external terminal members.

75 A furnace of this type is shown in Figure 4. The inner muffle 20 is preferably composed of a material having a high thermal conductivity as, for example, silicon carbide or fused alumina. The connector 21 is positioned in the rear wall of the furnace. The necessity of external terminal mountings in the rear of the furnace is thus eliminated.

80 By "siliconized silicon carbide" I mean any product wherein silicon carbide is impregnated or alloyed with silicon. These products vary somewhat in structure and constitution, depending upon the method of manufacture. A specific type of material which has been found to be very satisfactory is described in a copending application, United States Serial No. 382,004 filed July 29, 1929. 85 In the manufacture of the material in accordance with the process described in the above copending application, a heat hardened silicon carbide article, as for example one made by the process known as recrystallization, is surrounded with a small excess of molten silicon over that required for impregnation and the article and the surrounding silicon are then heated to a temperature at which the silicon rapidly vaporizes. The 90 heating is effected as rapidly as possible and the excess silicon is removed by vaporization. The original form of the article is preserved intact without the adherence of 95 globules of excess metal. After the excess silicon has been removed by vaporization, the article may be heated at a temperature above the boiling point of silicon for a very short time, usually about 30 seconds, in order to 100 secure a more complete alloying action. The 105 electrical resistance of the product is considerably decreased by the additional heating after the removal of the excess silicon metal.

110 The product as prepared above is believed to be an alloy of silicon and silicon carbide. Microscopic evidence indicates that the silicon dissolves the smaller particles of silicon carbide and also dissolves a portion of the 115 surface of the larger particles.

120 When siliconized silicon carbide connectors are employed in combination with silicon carbide resistors such as are sold under the trade name of "Globar", in which the terminal portions of the element are also sili- 125

conized, I have found that the arcing which takes place at high temperatures produces a slight welding action between the connector and the end portion of the resistor. This 5 weld does not have sufficiently great mechanical strength to interfere with the removal of the element, but it does produce a more effective electrical contact, and greatly minimizes any disintegration at the area of 10 contact from arcing.

Various forms and modifications of the connector above described may be used to meet particular conditions. By "connector" is meant any member which will afford electrical 15 connection between two or more resistors, and which can be placed entirely within an electric furnace.

I claim:

1. A siliconized silicon carbide connector 20 for rigid non-metallic resistors, the said connector having depressions adapted to receive the ends of the resistors.
2. A siliconized silicon carbide connector 25 for non-metallic resistors, the said connector having projections which are adapted to fit into corresponding cavities in the wall of an electric furnace.
3. In an electric furnace, a plurality of silicon carbide resistors and a connecting 30 member of siliconized silicon carbide within the furnace chamber.
4. In an electric furnace, a plurality of silicon carbide resistors and a connecting member of siliconized silicon carbide within 35 the furnace, said connecting member being positioned in a cavity within the inner wall of the electric furnace.
5. In an electric furnace, a plurality of silicon carbide resistors and a connecting 40 member of siliconized silicon carbide, the said connecting member being held in position by pressure transmitted through the resistor rods.
6. The method of electrically connecting 45 silicon carbide resistors which comprises forcing adjacent ends of two resistors against a connecting member of siliconized silicon carbide by resilient pressure.
7. The method of electrically connecting 50 non-metallic resistors which comprises connecting two resistors in series through an intermediary connecting member of siliconized silicon carbide.
8. The method of electrically connecting 55 silicon carbide resistors having siliconized ends, which comprises forcing the end of the resistor against a siliconized silicon carbide connecting member and effecting a temporary weld between the end of the resistor and the 60 said connecting member.

In testimony whereof I affix my signature.  
ALBERT H. HEYRÖTH.